# EUROPEAN PATENT SPECIFICATION

(11) **EP 0 188 747 B1**
(45) Date of publication and mention of the grant of the patent: **27.03.1991**
(21) Application number: 85115994.7
(22) Date of filing: 14.12.1985
(51) Int. Cl.: F41H 1/04

(54) **Caps of composite material for personal protection, such as helmets and the like**
Kopfbedeckung zum persönlichen Schutz aus Schichtmaterial, wie z.B Schutzhelme
Casque de protection en matériau composite

(30) Priority: 23.01.1985 IT 1921085
(43) Date of publication of application: 30.07.1986
(73) Proprietor: TECNO FIBRE S.p.A., 20121 Milano (IT)
(72) Inventor: Nocchi, Marzio, I-24030 Mozzo BG (IT); Cappa, Arnaldo, I-22079 Civello di Villaguardia CO (IT); Argentiero, Pietro, I-22079 Civello di Villaguardia CO (IT)
(74) Representative: Gioffreda, Fernando (IT)

(56) References cited:
- EP-A- 0 089 537
- FR-A- 2 425 046
- FR-A- 2 431 674
- GB-A- 1 367 403
- GB-A- 3 018 210
- US-A- 3 722 355
- US-A- 3 867 239

## Description

### Field of the Invention

The present invention relates to caps made of composite material for personal protection, such as helmets and the like, and more particularly to a composite helmets provided with high characteristics of resistance to the absorption of impact energy and to the dynamic to penetration by hard bodies, such as projectiles, splinters and the like.

### Description of the prior art

It is known that ballistic protective helmets (hereinunder also simply denominated as "helmets") are constituted by steel or other metal material. Such helmets have a limit of ballistic protection "V₅₀" of the order of magnitude of 1000-1200 feet/s (i.e., of about 305-366 m/s), wherein V₅₀ is the average of speeds measured for 10 impacts (projectile caliber 0.22, type 2), comprising the five lowest speeds for which the complete projectile penetration occurs, and the five highest speeds for which a partial penetration of projectile occurs, according to known MIL-STD-662B/1971 and MIL-P-46593A(ORD)/1962 (U.S.A.) standards, to which standards reference shall be made in the following disclosure when reference to ballistic characteristics and tests shall be made.

It is known that metal helmets show the drawback of being heavy (relatively to their ballistic characteristics), as well as of being good heat conductors, hence discomfortable when same helmets are to be borne over long time periods in very hot or very cold places.

Head coverings and helmets also exist (and are known) made of composite material, generally constituted by fiberglass (or of polyamide type) fabric, impregnated with a suitable resin, such as e.g. phenolic resins, thermosetting polyester resins, and others.

FR - A - 1,113,396 discloses, e.g., a composite product (useable for protective helmets too) constituted by an assembly (or laminate) of a plurality of sheets of fibrous matrial (fiberglass) impregnated with a synthetic resin (polyester), said sheets being linked to each other in a few contact points or areas, only, and wherein some of said sheets may be not resin-impregnated.

U.S. - A - 3,018,210 discloses in its turn a composite helmet (it too of non-metal materials) substantially having a "sandwich" structure, wherein two shells, respectively an inner and an outer shell, are both rigid (by being constituted by a resin-impregnated fibrous material), whilst an intermediate layer, comprised between said two shells, is constituted by a flexible not resin-impregnated ballistic fabric, wherein said layer is mostly free of moving between said outer and inner shells, which shells are solidly linked to each other by means of suitable linking means. FR-A-2,425,046 discloses a composite material for the personal protecon such as defined in the preamble of claim 1 and provided with high characteristics of resistance to the absorption of impact energy and to the dynamic penetration by hard bodies, comprising, in combination, an outer shell constituted by a metal material superimposed to an inner shell constituted by a composite laminate consisting of aromatic polyamide fibers impregnated with a synthetic resin, whereinsaid two shells are solidly linked to each other by means of polymeric material interposed between the said shells.

The composite material disclosed in this reference is characterized by a high total areal density and, therefore, it is not suitable for being used in the manufacture of caps such as helmets. More recently, non-metal helmets have been developed, essentially constituted by fibers with high physical-me-chanical characteristics (in particular, aramidic fibers, i.e., highly aromatic polyamide fibers), suitably woven, and assembled with synthetic resins. Said helmets are however very expensive, and moreover have ballistic properties (such as those hereinabove defined) around 2000 feet/s (about 610 m/s).

### Summary of the invention

Particular object of the present invention is hence to provide an improved composite ballistic helmet, not showing the above said drawbacks of the known art, and which is moreover provided with great resistance to the absorption of impact energy, as well as of greater resistance to penetration by projectiles, splinters, and the like.

Another object of the invention is to provide improved composite protective helmets for the most various uses, such as, e.g., helmets for miners, for operators of industrial plants, for firemen, for parachutists and the like.

According to the present invention, these and still other purposes, which shall be clear for those skilled in the art from the following detailed disclosure, are achieved by a cap of composite material for the personal protection, particularly a composi te helmet, provided with high characteristics of resistance to the absorption of impact energy and to the dynamic penetration by hard bodies, comprising, in combination, an outer shell constituted by a metal material superimposed to an inner shell constituted by a composite laminate consisting of aromatic polyamide fibers impregnated with a synthetic resin, wherein said two shells are solidly linked to each other by means of polymeric material interposed between the said shells, characterized in that the inner shell is constituted by fabrics made of aromatic polyamide fibers impregnated with a resin wherein said resin forms an elastic matrix with alveolar structure, the aromatic polyamide fiber of the fabrics being arranged into the alveoli of the alveolar structure.

### Detailed Disclosure of the Invention

Said outer metal shell is accomplished, according to the invention, by preferably using known steels for ballistic protective helmets, or deep-drawable aluminium alloys for ballistic use, whilst the fibrous matrial of said inner shell is preferably constituted by fabrics of fibers having high physical-mechanical characteristics, in particular polyamide fibers, fiberglass, and the like (the term "polyamide fibers" is intended to comprise also the polyamide fibers of aromatic type known as aramide fibers).

The above said outer metal shell has as its main function the absorbing and dissipating of the most of the impact energy of a projectile or of a splinter or the like, violently striking the same shell; the intermediate layer of polymeric material as above said (besides acting as the bonding agent between the two above said respectively outer and inner shells), cooperates with outer shell in absorbing and dissipating said impact energy, by delamination from the shell itself; finally, the inner shell as already indicated above has the function of absorbing the residual impact energy of the projectile or the like, by inner delamination, and moreover distributing said residual energy on a large surface, said shell being suitable (as a function of the type of fibrous material and of related impregnating resin selected to embody the invention) to delaminate, as well as to make said projectile to move along a trajectory not rectilineal, but tortuous (hence long), hence suitable to absorb much energy and to confer high resistance to penetration by the projectile.

The manufacturing of head coverings and helmets according to the invention is carried out by means of techniques of type known to those skilled in the art, such as cutting, deep drawing, moulding, lamination, polymerization, and the like.

It results evident from the above a complex and very efficacious action of resistance to impact and penetration by hard bodies (in particular, by projectiles) of the various components of composite helmet according to the invention, said action resulting of synergistic type, and however greater than that offered by a comparable helmet of known art, as it shall result more clearly from the Examples disclosed hereinunder.

A preferred, but not exclusive embodiment of the invention envisages that inner shell be constituted by the known"aramide ballistic fabrics" (provided with exceptionally high characteristics of tensile strength), and namely, in practice, e.g. by fabrics of Kevlar yarn (Trade mark of aromatic polyamide fiber by Du Pont de Nemours, E.I. & Co., U.S.A.), said fabrics being in a number of from 10 to about 15, and forming a thickness of about 4-6 mm, same fabrics being solidy assembled with each other by impregnation with a thermoplastic resin, e.g., polyethylene, or with a thermosetting resin, e.g., resins of modified phenol-formaldehyde type, vinyl esters, and polyesters.

The amount of resin represents about 15-35% (by weight, as dry solid matter) of the total of material constituting said inner shell (fibers + resin).

Always according to the said preferred embodiment, the layer of polymeric material interposed between the said outer and inner layers is constituted by a cellulose web of about 12 g/m², bonded with thermally melting adhesive on the basis of SIS (styrene-isoprene-styrene) copolymer.

Said layer can also be constituted by the same resin used to impregnate the inner layer. Other types of resin of known type which can be advantageously used are: modified melamine resins, polyester resins, vinyl resins, olefinic polymers and copolymers, as well as other known thermosetting resins and thermoplastic polymers.

The said intermediate layer of polymeric material (interposed between said two shells) can be accomplished, according to the invention, both as continuous layer (a cap, in particular a helmet, of "monolithic structure", being thus formed), as well as in other forms, as, e.g., a foam, a honeycomb structure, and the like, in that case a cap being formed with so-called "sandwich structure".

According to another embodiment, the invention envisages that inner shell be constituted by polyethylene sheets alternated to aramidic fiber fabrics, the polyethylene sheets forming (by partial bonding with each other through the interstices of said fabrics) an elastic matrix with alveolar structure, with function of tridimensional support, into the alveoli of which the filaments of aramidic fabrics are contained, freely encapsulated (see European Patent Application N° 0049014 A2, published), said polyethylene sheets and said fabrics being assembled with each other in the said alveolar mode by high-temperature pressing (e.g., under a pressure of about 5 kg/cm² at a temperature of about 165°C, and over a time of baout 15 minutes).

The alveolar structure as above said reacts elastically to projectile impact, as the filaments of aramidic fabrics cooperate harmonically in a very efficacious way in the impact area and in its surroundings, slightly sliding (by "controlled delamination") inside related alveoli, when said polyethylene alveolar structure is elastically deformed by the projectile.

The following Examples of invention embodiments, given to illustrative only and not limitative purposes, shall serve to better illustrate the same invention.

### Example 1

Ballistic helmet, so constituted:

- Outer shell: of steel sheet, type helmet M33 of Esercito Italiano (Italian Army), average thickness 1.1 mm;

- Inner shell: composite laminate constituted by 9 fabrics "TEXILAR", of 220 g/m² KEVLAR 49 fibers (TEXILAR = Trademark for fabrics by TEXINDUSTRIA S.p.a., Como), impregnated with a thermosetting resin of fire-proofed vinyl ester type;

- inner layer, interposed between the two said shells: made in form of cellulose web of 12 g/m² bonded with thermomelting adhesive on the basis of SIS (styrene-isoprene-styrene).

The weight per surface area unit of composite helmet (reported in plane) is of 10.8 kg/m² (of which, 8.8 kg/cm² the outer steel shell, and 2 kg/m² the inner shell + the intermediate layer).

The same helmet, submitted to the ballistic test according to the modalities already indicated at the beginning of the present disclosure, gives a value V₅₀ = 2350 feet/s (716 m/s).

The data of this example and of subsequent Examples are reported in Table 1 enclosed, in which to comparison purposes also the analogous data relating to known commercial helmets, of the type on the basis of Kevlar only and of steel only are reported.

### Example 2

Ballistic helmet constituted as that of Example 1, with the difference that the outer shell is of deep-drawable aluminium

alloys for ballistic use, average thickness 2.5 mm.

The weight per surface area unit of composite helmet (reported in plane) is of 10.8 kg/m² (of which, 6.5 kg/m² the shell of aluminium alloy, and 4.3 kg/m² the inner shell + the intermediate layer).

The limit of ballistic protection V₅₀ results equal to 2400 feet/s (732 m/s).

### Example 3

Ballistic helmet as that of Example 1, with the variant that the inner shell is constituted by a Kevlar-polyethylene laminate, with polyethylene formed according to an alveolar structure (as hereinabove disclosed), said laminate comprising 9 polyethylene films and 9 Texilar fabrics of 220 g/m² KEVLAR 49 fiber.

The weight per surface area unit of helmet (reported in plane) is of 10.8 kg/m² (of which, 8.8 kg/m² the steel shell, and 2 kg/m² the outer shell + the intermediate layer).

The limit of ballistic protection V₅₀ is equal to 2350 feet/s (716 m/s).

The above examples relate to helmets with outer shell respectively of steel and of aluminium alloy, but as already above said, such outer shell may be constituted, according to the invention, by any suitable metal material, such as e.g., titanium.

The present invention has been disclosed with particular reference to caps of composite material shaped for the protection of human head, but the protection area of the same invention is intended to enclose also caps shaped in different fashion, i.e., as shapes suitable to protect other parts of human body.

## Claims

1. Cap of composite material for the personal protection, particularly composite helmet, provided with high characteristics of resistance to the absorption of impact energy and to the dynamic penetration by hard bodies, comprising, in combination, an outer shell constituted by a metal material superimposed to an inner shell constituted by a composite laminate consisting of aromatic polyamide fibers impregnated with a synthetic resin, whereby said two shells are solidly linked to each other by means of polymeric material interposed between the said shells, characterized in that, the inner shell is constituted by fabrics made of aromatic polyamide fibers impregnated with a resin wherein said resin forms an elastic matrix with alveolar structure, the aromatic polyamide fiber of the fabrics being arranged into the alveoli of the alveolar structure.

2. Cap of composite material according to claim 1, wherein the resin is a thermoplastic or a thermosetting resin.

3. Cap of composite material according to claim 1, wherein the resin is constituted by polyethylene sheets.

4. Cap of composite material according to anyone of the preceding claims, wherein the laminate contains from 10 to 15 fabric layers.

5. Cap of composite material according to anyone of the preceding claims, wherein the amount of the resin is comprised from 15 to 35% by weight with respect to total weight of the inner shell.

6. Cap of composite material according to anyone of the preceding claims, wherein the polymeric material interposed between the two shells is a cellulose web coated with a termally melting adhesive.

7. Cap of composite material according to anyone of the preceding claims from 1 to 5, wherein the polymeric material interposed between the two shells is the same resin used to impregnate the inner layer.

8. Cap of composite material according to claims 7, wherein the polymeric material interposed between the two shells is in the form of a honeycomb structure.

## Revendications

1. Coiffure en matériau composite pour la protection individuelle, particulièrement casque en matériau composite doté de fortes caractéristiques de résistance à l'effet de choc et à la force de pénétration de corps solides, comprenant, en combinaison, une coque externe constituée d'un matériau métallique, superposée à une coque interne consistant en un matériau laminé composite stratifié à base de fibres de polyamide aromatique imprégnées d'une résine synthétique, de manière que lesdites deux coques soient solidement réliées l'une à l'autre au moyen de matériau polymère interposé entre lesdites coques, caractérisée en ce que la coque interne consiste en tissu à base de fibres de polyamide aromatique imprégnées d'une résine, ladite résine formant une matrice élastique à structure alvéolaire, les fibres de polyamide aromatique du tissu étant disposées dans les alvéoles de la structure alvéolaire.

2. Coiffure en matériau composite selon la revendication 1, dans laquelle la résine est une résine thermoplastique ou thermodurcissable.

3. Coiffure en matériau composite selon la revendication 1, dans laquelle la résine consiste en feuilles de polyéthylène.

4. Coiffure en matériau composite selon l'une quelconque des revendications précédentes, dans laquelle le matériau composite stratifié comporte de 10 à 15 couches de tissu.

5. Coiffure en matériau composite selon l'une quelconque des revendications précédentes, dans laquelle la quantité de résine est comprise entre 15 et 35% en poids par rapport au poids total de la coque interne.

6. Coiffure en matériau composite selon l'une quelconque des revendications précédentes, dans laquelle le matériau polymère interposé entre les deux coques est un tissé de cellulose recouvert d'un adhésif thermofusible.

7. Coiffure en matériau composite selon l'une quelconque des revendications 1 à 5, dans laquelle le matériau polymère interposé entre les deux coques est la même résine que celle utilisée pour imprégner la couche interne.

8. Coiffure en matériau composite selon la revendication 7, dans laquelle le matériau polymère interposé entre les deux coques se présente sous la forme d'une structure en nid d'abeilles.

## Patentansprüche

1. Kopfbedeckung aus Verbundwerkstoff zum persönlichen Schutz, insbesondere Helm aus Verbundstoff, mit hohen Widerstandswerten gegenüber Absorption von Schlagenergie und dynamischer Durchdringung durch Hartkörper, umfassend, in Kombination, eine äußere Schale aus metallischem Material, die sich über einer inneren Schale befindet, die aus einem Schichtstoff-Verbundstoff aufgebaut ist, der aus aromatischen Polyamidfasern besteht, die mit einem synthetischen Harz imprägniert sind, wobei diese Schalen mittels eines polymeren Materials, das sich zwischen besagten Schalen befindet, fest miteinander verbunden sind, dadurch gekennzeichnet, daß die innere Schale aus Geweben aus aromatischen Polyamidfasern aufgebaut ist, die mit einem Harz imprägniert sind, wobei das Harz eine elastische Matrix mit zellenförmiger Struktur bildet und die aromatischen Polyamidfasern der Gewebe die Zellen der zellförmigen Struktur bilden.

2. Kopfbedeckung aus Verbundwerkstoff nach Anspruch 1, worin das Harz ein Thermoplast oder ein härtbares Harz ist.

3. Kopfbedeckung aus Verbundwerkstoff nach Anspruch 1, worin das Harz aus Polyethylenfolien aufgebaut ist.

4. Kopfbedeckung aus Verbundwerkstoff nach irgendeinem der vorhergehenden Ansprüche, worin das Laminat 10 bis 15 Gewebeschichten enthält.

5. Kopfbedeckung aus Verbundwerkstoff nach irgendeinem der vorhergehenden Ansprüche, worin die Menge an Harz, bezogen auf das Gesamtgewicht der inneren Schale 15 bis 35 Gew.-% umfaßt.

6. Kopfbedeckung aus verbundwerkstoff nach irgendeinem der vorhergehenden Ansprüche, worin das polymere Material, das sich zwischen den zwei schalen befindet, ein Cellulosenetz ist, das mit einem unter Einwirkung von Wärme schmelzenden Klebstoff beschichtet ist.

7. Kopfbedeckung aus Verbundwerkstoff nach irgendeinem der vorhergehenden Ansprüche 1 bis 5, worin das polymere Material, das sich zwischen den zwei Schalen befindet, dasselbe Harz ist, das zur Imprägnation der inneren Schicht verwendet wird-

8. Kopfbedeckung aus Verbundwerkstoff nach Anspruch 7, worin das polymere Material, das sich zwischen den zwei Schalen befindet, in Form einer Bienenwabenstruktur vorliegt.
